

Dec. 13, 1966

F. A. BIRIBAUER ET AL

3,291,718

## COMBINATION LUBE PROCESS

Filed March 16, 1965



Frank A. Birbauer  
James D. Bushnell  
Harold N. Weinberg

## Inventors

By *Perry Carvelas* Patent Attorney

## 1

3,291,718

## COMBINATION LUBE PROCESS

Frank A. Biribauer, Cranford, James D. Bushnell, Berkley Heights, and Harold N. Weinberg, East Brunswick, N.J., assignors to Esso Research and Engineering Company, a corporation of Delaware

Filed Mar. 16, 1965, Ser. No. 440,155

17 Claims. (Cl. 208—36)

This invention is directed to an improvement in the manufacture of lubricating oils. More particularly, the invention teaches a process whereby paraffinic and naphthenic lubes may be produced from non-naphthenic crudes while substantially increasing lube yield per barrel of crude over that obtained in conventional processing. This is accomplished by utilizing a unique sequence of residuum treating in conjunction with an unexpected synergistic extraction effect of treating an atmospheric residuum in a combination tower and a heart-cut tower.

Two types of crude oil are normally utilized in the manufacture of lubes. Paraffinic crudes are generally used in the production of high quality motor oils, aviation and turbine oils. This type of crude includes fraction which have a relatively high viscosity index which can be substantially increased by treating. The other crude type, naphthenic crude is used to make large volumes of lubes in which the viscosity index is not of great importance. The outstanding feature of these crudes is that they make lubricants which have especially desirable properties in certain heavy duty engines such as the diesel engine.

It is well known in the art to treat feed oils, particularly distillate feed oils, with various solvents in order to separate the relatively more aromatic type constituents having low V.I. from the relatively more paraffinic type constituents having high V.I. extraction solvents generally employed are phenol, various cresols, furfural, sulfur dioxide and the like. In these operations the feed oil is usually contacted with the selected solvent such as phenol, either in a countercurrent treating operation or in a multi-stage batch operation under temperature and pressure conditions to secure phase separation. As a matter of practice, the oil to be treated is usually introduced into one end of a countercurrent treating zone while the solvent or solvent mixture is introduced at the other end. The solvent and oil flow countercurrently under temperature and pressure conditions whereby phase separation is secured. The solvent rich or solvent extract phase is withdrawn from one end of the countercurrent treating zone, while the solvent poor or the raffinate phase, comprising the more paraffinic type constituents, is withdrawn from the other end of the treating zone. The respective streams are then handled in a manner to separate the solvent from the oil. It is further known to those skilled in the art to conduct a light hydrocarbon deasphalting process. In such a process, an oil phase or feed stream containing asphaltic type constituents is mixed with a light hydrocarbon solvent such as, for example, liquid propane, under temperature and pressure conditions whereby the asphaltic type constituents are precipitated. After separation of the asphaltic type constituents from the deasphalting oil, the respective streams are handled in well known manners to recover the solvent.

Waxy constituents are also removed from paraffinic type oils in order to improve the quality of the oil itself. This improvement in quality is represented by a deduction

## 2

of the cloud and pour point of the oil. This is accomplished by well known methods which employ a dewaxing solvent such as propane, methyl ethyl ketone or similar product. In operations of this type, the waxy oil and the solvent are usually heated to a temperature to secure a single phase or substantially complete miscibility of the ingredients. The waxy mixture is then chilled in order to precipitate wax particles or crystals from the solution. The chilled mass is filtered in order to segregate the wax particles and further handled in a manner to recover the dewaxed solvent.

These processes and others like them in which the various steps are combined, have represented a substantial step forward in the art. However, several serious drawbacks do exist with the processes which are currently in use. First, naphthenic lubes can only be made from naphthenic type crudes. Second, the yield of high V.I. paraffinics for the best quality motor and aviation oils is not as high as is desirable. By viscosity index is meant the relative measure of the difference in viscosity at 100° F. and 210° F. A high viscosity index means a small change in viscosity with temperature which is desirable in a motor oil. In general, removal of aromatic type compounds by extraction improves the viscosity index. According to this invention these problems have now been solved by making use of unexpected synergistic effect found in a combination lube process. Naphthenic and paraffinic lubricating oils are prepared from an atmospheric residuum by introducing the residuum into a combination treating zone. A solvent having a preferential selectivity for aromatic type constituents as compared to paraffinic type constituents is introduced into the upper region of this combination zone. A deasphalting solvent is introduced into the lower area of the combination zone. A deasphalted raffinate phase is removed from the top region of a combination zone. This raffinate is then passed to a heart-cut tower zone. A solvent having a preferential selectivity for aromatic type constituents as compared to paraffinic type constituents is introduced into the heart-cut zone. A raffinate phase comprising paraffinic type constituent is withdrawn from the top of the heart-cut tower and the extract phase comprising naphthenic type constituent is withdrawn from the bottom region from the tower zone. This is the result of an unexpected synergistic effect which has been discovered and paraffinic as well as naphthenic lubes are produced from non-naphthenic crudes. In addition, yields are increased.

The first process unit in the combination lube process is a vacuum flash tower where feed which is usually an atmospheric residuum is introduced. Steam stripping is used to effect efficient fractionation to reject light ends not required for lube manufacture. The stripped residuum is then cooled before entering the combination tower. The feed enters at a temperature of about 100° F. to 150° F. Feed entry may be at many different points along the wall of the tower but it is preferred to introduce the feed close to the center of the tower, propane or another suitable deasphalting agent such as butane, pentane or ethane enters the bottom of the tower at a temperature of about 100° F. to 150° F. The propane acts as an asphalt precipitator. Phenol or furfural nitrobenzene dichlorated ether, phenol, cresol mixtures enters the top of the tower and performs an extraction of low viscosity index, poor color, highly aromatic components from the feed. The raffinate phase from the combination tower is typically

40 to 60% of the feed. This raffinate phase includes a high V.I. oil containing the majority of the treat propane from the combination tower and some dissolved phenol. The majority of the propane is then flashed in a drum at high temperatures and pressures. The bottoms from this drum contain the phenol and oil from the combination tower raffinate and a small amount of propane. The extract phase leaving the combination tower contains the bulk of the phenol, the remainder of the propane, the precipitated asphalt, and the highly aromatic extracted oil. The extract phase is sent to a high pressure flash drum where the bulk of the propane is recovered. The bottoms from this flash drum contain the phenol, asphalt and extract.

The raffinate phase oil and phenol mixture from the high pressure propane flash next enters a second extractor referred to hereinafter as the "heart-cut" extractor. Here, additional phenol is added to effect the separation of high V.I. paraffinic type oils and medium V.I. industrial type oils. The raffinate from the heart-cut extractor is then stripped of all solvents in a solvent recovery tower. The phenol and propane are vaporized and the high quality oil is stripped with a volatile stripping gas, which may be propane, to completely recover all solvent. The raffinate oil is then sent to a vacuum rerun tower where products are cut to desired viscosity grades. Typically, light, intermediate, and heavy viscosity distillates and a residual bright stock are obtained in the paraffinic rerun tower. Steam stripping may be used on side streams for flash correction to remove any propane and high vapor pressure, low boiling components remaining in any of the side streams. The side streams are cooled and sent to intermediate tankage. The bottoms from the rerun tower are hydrofined while hot to reduce Conradson carbon and to improve color and color stability. The hydrofined bright stock is cooled and sent to intermediate tankage. Some or all of the distillates may also be hydrofined if required for product quality. The extract phase from the heart-cut extraction tower enters a solvent recovery tower similar to that used on the heart-cut raffinate. The heart-cut extract contains 60 to 90% of the treat phenol and the oil yield is typically from 20 to 50% of the feed to the heart-cut extractor. This oil-phenol mixture is heated by exchange with hot rerun side streams and with condensing phenol.

The propane stripping gas is used in the bottom section of the solvent recovery tower to completely remove all phenol. The phenol stripped hot oil is then hydrofined or treated in any desired manner such as caustic rerunning acid treating or clay treating as a broad cut to improve the color and color stability of the naphthenic stocks. The hydrofined product then passes through a furnace where it is heated to a desired temperature before entering a vacuum rerun tower. Light, medium and heavy viscosity distillate stocks are cut from the naphthenic oil. A residual naphthenic bright stock may also be recovered if desired. Steam stripping is used in the bottom to effect efficient fractionation and provide reasonable yields of high viscosity material. These stocks pass through side stream strippers which steam strip out any entrained solvent and improve fractionation. Each side stream is then cooled by exchanging with the extract phenol mixture from the heart-cut tower. The side streams are then trim cooled to 160° F. to 200° F. before going to intermediate tankage. The bottoms from the naphthenic rerun tower is similarly cooled before going to tankage. The combination tower extract, approximately 50% of the feed, contains asphalt and highly aromatic distillate oil. The extract also contains 50 to 75 volume percent propane on oil and 50 to 90% of the treat phenol. This extract is heated and flashed at 500° F. to 600° F. and 225 to 300 p.s.i.g. to remove the bulk of the propane, approximately 90%. The oil-propane phenol mixture is then heated in a furnace to vaporize the remainder of the solvent. The solvent-free extract is stripped with propane stripping gas

to completely recover the phenol. This stripped asphalt aromatic oil portion enters a vacuum stripper to remove the last traces of propane and phenol. This tower acts as an explosivity corrector. The propane and phenol streams from the heart-cut raffinate solvent recovery tower, the heart-cut extract solvent recovery tower and combination tower extract solvent recovery tower are combined and utilized as a source of high level heat. The condensing phenol and sensible heat available in this stream is utilized as preheat for each of the solvent recovery towers. The condensed phenol and propane are trim cooled before entering a phenol accumulator drum. This drum operates at 20 to 75 p.s.i.g. and 200° F. to 275° F. Vapor is withdrawn from the phenol accumulator which contains 5 to 15% phenol with the remainder being propane on other light hydrocarbon solvent. This stream is cooled to 115° F. to 125° F. to condense the remainder of the phenol and recover essentially phenol-free propane vapors. These propane vapors go to a propane compressor knockout drum where they are mixed with the chilled propane from the dewaxing plant. A common propane compressor is used to compress the stripping gas and vaporized combination tower treat propane and the chilled propane required for the dewaxing plant. These vapors are condensed at 150° F. to 125° F. and 250 to 275 p.s.i.g. The stripping gas required for the solvent recovery towers is withdrawn at an intermediate stage of the propane compressor. Makeup propane required for combo tower treat is removed from the propane accumulator. Dewaxing plant propane is also withdrawn from this drum. The paraffinic and naphthenic lubes are dewaxed in block operation. Each stock is individually dewaxed in a propane dewaxing plant. The paraffinic stocks have a yield of 75 to 70% dewaxed oil and the naphthenic stocks have a yield of 85 to 95% dewaxed oil. The pour point of the finished products decreases with decreasing yield and may be varied from 0° F. to 30° F. in the dewaxing plant. The dewaxed stocks are sent to product tankage and serve as base stocks for finished motor oils and industrial oils. The combination lube plant provides broad cut continuous processing of an atmospheric residuum of a variety of viscosities and qualities.

The figure is a schematic view of a preferred embodiment of the instant invention.

Turning to the figure an atmospheric residuum containing the full range of lubricating oils from light distillate to bright stock, which is a residuum from a typical Mid-East crude is introduced through line 1 into tower 2.

Atmospheric bottoms may be used directly if the residuum length is suitable. However, stripping is often required to remove light material which is not required for lube manufacture. These light materials are typically boiling below 650° F. Tower 2 is a stripping tower which operates under vacuum. The tower would be operated at a pressure of 100 to 300 mm. Hg and a temperature of 650° F. to 750° F. Overhead products are removed through line 3. This accounts for about 10 LV percent of the total residuum introduced into the stripping tower. The stripout may be returned as distillate to the fuel side of a refinery or utilized as fuel for the plant of the instant invention.

The bottoms from the stripping tower 2 are removed through line 4 and fed to combination tower 5. The feedstock is introduced at approximately the middle of the combination tower. Phenol is injected into the top region of the tower through line 6 at a temperature of 120° F. to 200° F. and a treat feed rate of 50 to 150% on feed. Liquid propane is injected into the bottom of the tower 7 at a temperature of 120° F. to 200° F. and a treat rate of 300 to 500% on feed. Tower pressure is adjusted to maintain propane in the liquid phase, generally 300 to 500 p.s.i.g.

The overhead product from the combination tower removed through line 8 is a deasphalted raffinate phase consisting of the more paraffinic portion of the residuum, a

major portion of the solvent propane and a minor portion of the phenol. About 80 to 100% of the propane, about 30 to 40% of the phenol and about 40 to 60% of the more paraffinic portion of the residuum are passed overhead. The more paraffinic portion of the residuum will typically have a V.I. in the range of 60 to 100. The bottoms from the material treated within the combo tower 5 is an extract phase containing the more asphaltic and aromatic portion of the residuum, a major portion of the phenol and a minor portion of the solvent propane. This material is sent to a solvent recovery facility 10 through line 9 where the phenol and propane are recovered through line 11. An alternate possibility, although it is not shown in drawing, is the recovery of the solvent by heating and stripping. The asphaltic, aromatic portion of the residuum is a high viscosity, low V.I., low API gravity material. This is removed through line 12. It may be used as fuel or processed further to recover potentially by-products such as highly aromatic specialty oils and asphalt.

The overhead material from the combo tower 5 is removed through line 8 and sent to solvent recovery facilities 13 where most of the propane is recovered through line 14 for reuse elsewhere. The propane is recovered by heat flashing or any other suitable means. Phenol remains with the deasphalted raffinate oil and is removed through the bottom of recovery facilities 13 through line 15.

The deasphalted raffinate oil phase, containing about 45 volume percent oil, 40 to 45% phenol and about 10 to 15% propane, is introduced at substantially the mid point of heart-cut tower 16. Heart-cut tower 16 is a tower designed to remove a select portion of a middle distillate. No intermediate tankage is required between combination tower 5 and heart-cut tower 16. The oil plus phenol stream is introduced to the heart-cut tower at a temperature range of 120° F. to 200° F. Phenol is introduced near the top of heart-cut tower 16 at a treat rate in the range of 20 to 200%; this is based on the deasphalted raffinate oil feed, and at a temperature of 120° F. to 200° F.

The overhead from the heart-cut tower is removed through line 18. It is a raffinate phase consisting of the highest V.I. components of the feed oil, a minor portion of the phenol and a small amount of residual propane from the combo tower 5. The bottoms from the heart-cut tower are removed through line 19. This is an extract phase consisting of medium and lower V.I. components of the feed oil. A major portion of the phenol is also included as well as a small amount of propane. The higher V.I. raffinate portion of the feed oil which is subsequently processed to make paraffinic lubes is typically in the range of 90 to 105 V.I. The medium and lower V.I. extract portion of the feed oil, which is subsequently processed to make naphthenic lubes, is typically in the range of 30 to 80 V.I. It has unexpectedly been found that the small amount of propane in the feed to the heart-cut extraction step is desirable. This desirability is for a variety of reasons. Initially, the propane reduces the viscosity of the phases, thus permitting easier settling in the extraction tower. However, a further and also unexpected result occurs in that the presence of propane favorably alters the solubility of relationships between phenol and oil, permitting a better quality oil to be made with less phenol treat and at lower temperature.

The high V.I. overhead from the heart-cut tower 16 is removed through line 18 from whence it is sent to solvent recovery facilities 20 where phenol and residual propane are removed for reuse. Their removal is effected through line 21. This represents all of the remaining phenol and propane. The solvent-free raffinate oil is removed from the bottom of tower 20 through line 22 from whence it is passed to vacuum fractionating column 23 for distillation into viscosity grades as required by the individual product slates. The temperature in the vacuum fractionating column 23 varies between 650° F. and

750° F., pressure within the column varies between 50 to 200 mm. Hg. Three distillate grades are removed from the column 23. A light grade is removed through line 24, a medium grade through 25 and a heavy grade through line 26. It would be obvious to one skilled in the art that more or fewer grades may be made depending on the product lube slate and/or requirements of the individual plant. If desired, the distillate grade may be stored in tankage and then sent to a dewaxing plant 27 in block operation.

Bottoms from the vacuum fractionating tower 23 is hydrofined in reactor 29. The bottoms are passed through line 28 into the hydrofiner 29. It is, of course, obvious that any lube finishing apparatus may be utilized and that the hydrofining apparatus is merely convenient. Distillates may also be hydrofined if required for product quality. Typical lube hydrofining conditions are utilized. These include a space velocity of .2 through 2.0 volumes of liquid feed per volume of catalyst per hour, pressures of 500 to 1000 p.s.i.g., temperatures of 450° F. to 650° F. and treat gas rates of 200 to 2000 s.c.f./barrel of feed. Hydrofining takes place over a cobalt molybdate catalyst. This hydrofining treatment improves the color and color stability of the vacuum fractionating tower bottoms and reduces carbon residue. The hydrofined bright stock is stored in tankage and charged to the dewaxing unit 27, in blocked operation and then sent to finished lube base stock tankage. Dewaxing may be carried out in conventional fashion using ketone, propane urea, spray or any other suitable process.

Low to medium V.I. bottoms from the heart-cut tower 16 are passed through line 19 from whence they are sent to solvent recovery zone 31. Phenol is removed through line 32 so that it may be reused. The solvent-free extract oil is removed through line 33 and sent to hydrofiner 34. Conditions within hydrofiner 34 are similar to those within hydrofiner 29. No intermediate tankage is required between the heart-cut tower and the hydrofiner. The hydrofined extract oil is removed from the bottom of hydrofiner 34 through line 35 and sent to vacuum fractionating column 36. The vacuum fractionating column is maintained at a temperature of 650° F. to 750° F. and a pressure of 50 to 200 mm. Hg. Three distillate grades are made and they are recovered through lines 37, 38 and 39. A light grade is recovered through line 37, a medium grade through line 38 and a heavy grade through line 39. Needless to say, more or fewer grades may be recovered depending on the product lube slate. These are naphthenic base stocks. The lubes in lines 37, 38 and 39 may be stored or sent directly to dewaxing zone 27. Dewaxing zone 27, as mentioned previously is any suitable dewaxing process. Desired naphthenic base stocks are then recovered through lines 37', 38' and 39' after the dewaxing in zone 27.

The combo lube plant processing sequence described in the drawing may be altered to fit special circumstances. For example, it may be economical to place dewaxing upstream of rerunning which would reduce the number of intermediate tanks required and would make it possible to operate with only one rerun tower. A single rerun tower could be used, even in the preferred embodiment of the drawings, if appropriate tankage is provided upstream to block the paraffinic and naphthenic broad cuts through. These variations in sequence and equipment requirements are well within the scope of the combo lube process of the instant invention.

The combo lube plant processing conditions can be altered to make a variety of products from widely different crudes. Combo tower temperatures and solvent treats may be adjusted to handle a wide variety of crude residua and make raffinate suitable for processing to meet different lube product slates. For example, the typical effect of increasing combo tower temperature is to decrease raffinate oil yield while improving viscosity index, carbon residue and color; or alternatively, to permit using lower

phenol treats. Increasing phenol treat generally has similar effects to increasing tower temperature. When propane treats are increased, the effect on raffinate oil is usually to increase yield, to decrease carbon residue and viscosity index and to improve color.

TABLE I.—SAME COMBO TOWER TREATING CONDITIONS HANDLE WIDELY DIFFERENT CRUDES

|                               | 75%<br>Aramco<br>25%<br>Safaniya | Canadian<br>Seco | U.S.<br>Coastal |    |
|-------------------------------|----------------------------------|------------------|-----------------|----|
| Reduced Crude Feed:           |                                  |                  |                 |    |
| Gravity, ° API                | 13.2                             | 16.5             | 20.2            |    |
| Viscosity, SSU/210            | 315                              | 842              | 82              | 15 |
| Conradson Carbon, Wt. Percent | 12.2                             | 9.8              | 2.4             |    |
| Combo Tower Conditions:       |                                  |                  |                 |    |
| Propane Treat, Vol. Percent   | 420                              | 400              | 440             |    |
| Phenol Treat, Vol. Percent    | 100                              | 100              | 105             |    |
| Temp., ° F., Top/Bottom       | 145/125                          | 145/125          | 125/110         |    |
| Combo Tower Raffinate:        |                                  |                  |                 |    |
| Yield, Vol. Percent           | 52                               | 60               | 85              |    |
| VI (dewaxed)                  | 91                               | 80               | 59              |    |
| Viscosity, SSU/210            | 69                               | 108              | 67              |    |
| Gravity, ° API                | 26.4                             | 26.7             | 23.4            |    |
| Conradson Carbon, Wt. Percent | 0.7                              | 0.6              | 0.5             |    |

The above table indicates the variety of crudes which this invention can treat. Paraffinic crudes such as Aramco/Safaniya, naphthenic crudes such as U.S. Coastal and mixed base crudes such as Canadian Seco may all be successfully treated. Desirable results may be obtained by treating this variety of crudes as illustrated by the combo tower raffinate analysis. The yields of 52 volume percent, 60 volume percent and 85 volume percent are high. The V.I.'s and other characteristics of the raffinate are suitable for further processing in the heart-cut tower to make high V.I. paraffinics and medium V.I. naphthenics.

#### Example

An Aramco Safaniya atmospheric residuum which was 75% Aramco and 25% Safaniya was introduced into a processing apparatus essentially as described in the attached figure. About 1000 barrels were introduced into a combination tower. The tower was maintained at a temperature of 125° F. to 145° F. and a pressure of 440 p.s.i.g. About 4680 barrels of deasphalted raffinate phase were withdrawn from the top of the tower. This included about 3900 of propane and about 280 of phenol. Most of the propane was removed in a solvent recovery facility and the raffinate and phenol and residual propane were passed to a heart-cut tower. The temperature in the heart-cut tower was 145° F. to 150° F. and the pressure was 220 p.s.i.g. An overhead was recovered from the heart-cut tower, this consisted of about 470 barrels of raffinate phase containing the raffinate oil having a V.I. of 101. The bottoms from the heart-cut tower were an extract phase containing medium and lower V.I. components having a V.I. of 60. About 810 barrels of extract phase were recovered from the bottom of the tower. The overhead fraction was treated in a solvent recovery wherein phenol and residual propane were removed. About 350 barrels of solvent-free raffinate oil were then sent to a vacuum fractionating column wherein the temperature was 730° F. and the pressure was 63 mm. Hg. Three distillate grades of paraffinic lubes were removed from this vacuum fractionating column. They were 6 barrels of overhead discard, 45 barrels of low viscosity oil, 48 barrels of intermediate viscosity oil and 155 barrels of high viscosity oil. The bottoms from the vacuum fractionating column comprising 96 barrels were hydrofined at 625° F., 800 p.s.i.g. and 500 s.c.f. per barrel hydrogen treat rate. The bottoms from the heart-cut tower, constituting about 810 barrels were sent to a solvent recovery zone wherein propane and phenol were removed. The extract oil comprising 150 barrels was

then sent to a hydrofiner. The temperature within the hydrofiner was 625° F., the pressure was 800 p.s.i.g. and the hydrogen treat rate was 500 s.c.f./bbl. The catalyst was cobalt molybdate. The hydrofined extract oil was then sent to a vacuum fractionating column wherein the temperature was 696° F. and the pressure 63 mm. Hg. Three streams of naphthenic crudes were removed from the vacuum fractionating column. There were 3 barrels of overhead discard, 15 barrels of low viscosity oil, 35 barrels of medium viscosity oil and 77 barrels of high viscosity oil. All the streams, both paraffinic and naphthenic, were then subjected to propane dewaxing.

The combo lube process produces paraffinic and naphthenic lubes from non-naphthenic crudes, maximizes lube yield per barrel of crude, provides considerable flexibility to vary lube product distribution with product slate requirements and reduces lube plant costs compared with conventional processing.

Although this invention was described with some particularity, it is intended only to be limited by the attached claims.

What is claimed is:

1. In a process for the production of naphthenic and paraffinic lubricating oils from a paraffinic atmospheric residuum which comprises introducing the said atmospheric residuum into a combination treating zone, introducing a solvent having a preferential selectivity for aromatic-type constituents as compared to paraffinic-type constituents into the upper area of said combination zone,

30 introducing a deasphalting solvent into the lower area of said combination zone, removing a deasphalted raffinate phase from the top region of the said combination zone, passing said raffinate to a heart-cut tower zone, introducing a solvent having a preferential selectivity for aromatic-type constituents as compared to paraffinic-type constituents into the said heart-cut tower zone, withdrawing

35 a raffinate phase comprising paraffinic-type constituents from the top of said heart-cut tower, withdrawing an extract phase comprising naphthenic-type constituents from the bottom region of said tower zone.

2. The process of claim 1 wherein said solvent having a preferential selectivity for aromatic-type constituents is phenol and said deasphalting solvent is propane.

3. The process of claim 2 wherein said combination zone is maintained at a temperature of 120° F. to 200° F. and a pressure of 300 to 500 p.s.i.g., and the said heart-cut zone is maintained at a pressure of 200 to 400 p.s.i.g. and a temperature of 120° F. to 200° F.

4. The process of claim 1 wherein said atmospheric residuum is a residuum from a paraffinic crude.

5. A process for the production of naphthenic and paraffinic crudes from a paraffinic atmospheric residuum which comprises preflashing hot atmospheric residuum to reject light ends, passing the light ends free residuum into a combination tower zone, introducing a solvent having a preferential selectivity for aromatic-type constituents as compared to paraffinic-type constituents into the upper area of said tower zone, introducing a deasphalting solvent into the lower area of said tower zone, withdrawing an overhead fraction containing desired lube components, passing said overhead fraction to a heart-cut tower zone, recovering two fractions from the said heart-cut tower zone, an overhead fraction rich in paraffinic lube constituents and a bottoms fraction rich in naphthenic lube constituents, passing the overhead fraction to a vacuum fractionating tower wherein it is separated into a plurality of streams, passing said plurality of streams to a dewaxing zone and recovering high quality paraffinic lube constituents, passing said bottoms fraction from heart-cut tower to a hydrotreating zone, passing said hydrotreated fraction to a vacuum fractionation zone, whereby said fraction is divided into a plurality of naphthenic streams, passing said naphthenic streams to a dewaxing zone and recovering a plurality of naphthenic lube streams.

6. The process of claim 5 wherein said hydrotreater

is maintained at a temperature of 500° F. to 650° F., a pressure of 500 to 1000 p.s.i.g. and a hydrogen treat rate of 200 to 1000 s.c.f.

7. The process of claim 5 wherein the said solvent having a preferential affinity for aromatic-type constituents is phenol and the said deasphalting solvent is propane.

8. The process of claim 5 wherein the said heart-cut tower is maintained at a temperature of 120° F. to 200° F. and a pressure of 200 to 400 p.s.i.g.

9. The process of claim 5 wherein the said combination tower is maintained at a temperature of 120° F. to 200° F. and a pressure of 300 to 500 p.s.i.g.

10. The process of claim 5 wherein the said overhead fraction from the seed heart-cut tower zone and the said bottom fraction from the said heart-cut tower zone are both subjected to solvent recovery before being treated further.

11. An improved process for producing both paraffinic and naphthenic lubes which comprise passing an atmospheric bottoms feed to a stripping zone wherein light components are removed, passing the bottoms from said stripping zone to a combination tower zone, passing phenol into the top region of the said tower zone, passing propane into the bottom region of said tower zone, removing a raffinate from the top region of said tower zone, passing said raffinate to a solvent recovery zone wherein at least a portion of the said propane is removed, passing the said propane poor raffinate to a heart-cut tower zone, introducing phenol into the top region of said heart-cut tower zone, removing a paraffinic lube constituent from the top region of said tower zone, removing a naphthenic-type lube constituent from the bottom region of said tower zone, passing said paraffinic constituent to a solvent recovery zone wherein at least a portion of the phenol and at least a portion of the propane are removed, passing the said propane and phenol poor paraffinic constituent into a vacuum fractionating zone from whence a plurality of streams are removed, passing said plurality of streams to a dewaxing zone from whence a plurality of high quality paraffinic streams are recovered, passing the said naphthenic con-

stituent to a solvent recovery zone wherein at least a portion of the said phenol is removed, passing the said phenol poor naphthenic constituent to a hydrotreating zone, removing the hydrotreated naphthenic constituent and passing it to a vacuum fractionating column from whence a plurality of naphthenic streams are removed, passing the naphthenic streams into a dewaxing zone, withdrawing said plurality of high quality naphthenic streams from the dewaxing zone.

12. The process of claim 11 wherein the said hydrotreating takes place over a cobalt-molybdate catalyst at a temperature of 500° F. to 650° F. and a pressure of 500 to 1000 p.s.i.g.

13. The process of claim 11 wherein the said atmospheric bottom feed is recovered from a paraffinic crude.

14. The process of claim 11 wherein the said dewaxing is propane dewaxing.

15. The process of claim 11 wherein the said combination tower is maintained at a temperature of 120° F. to 200° F. and a pressure of 300 to 500 p.s.i.g.

16. The process of claim 11 wherein the said heart-cut tower is maintained at a temperature of 120° F. to 200° F. and a pressure of 200 to 400 p.s.i.g.

17. The process of claim 11 wherein the said vacuum fractionating columns are maintained at a temperature of 650° F. to 750° F. and a pressure of 50 to 300 mm. Hg.

#### References Cited by the Examiner

#### UNITED STATES PATENTS

|    |           |         |                 |         |
|----|-----------|---------|-----------------|---------|
| 30 | 2,095,972 | 10/1937 | Faragher        | 208—314 |
|    | 2,168,875 | 8/1939  | Noll            | 208—317 |
|    | 2,687,982 | 8/1954  | Baumann         | 208—34  |
|    | 2,692,222 | 9/1954  | Packie          | 208—34  |
| 35 | 2,764,529 | 9/1956  | Leygonie et al. | 208—19  |
|    | 3,052,622 | 9/1962  | Johnson et al.  | 208—27  |

DELBERT E. GANTZ, Primary Examiner.

HERBERT LEVINE, Examiner.